

## UNITED STATES PATENT OFFICE

LEON McCULLOCH, OF PITTSBURGH, PENNSYLVANIA, ASSIGNOR TO WESTINGHOUSE ELECTRIC & MANUFACTURING COMPANY, A CORPORATION OF PENNSYLVANIA

## COMPOSITION OF MATTER

No Drawing.

Application filed May 31, 1930. Serial No. 458,895.

My invention relates to compositions of matter and more particularly to insulating or friction material which is coherent at high temperatures.

5 The principal object of my invention is to provide a composition of matter comprising asbestos and an inorganic binder that is non-volatile at high temperatures.

Another object of my invention is to provide 10 an insulating or friction material comprising asbestos, an organic binder and chromic sulphate.

A further object of my invention is to provide 15 a process of producing a coherent mass of asbestos which comprises impregnating asbestos fibers with an aqueous solution of chromic sulphate, either alone or with organic binders, and heating the impregnated material at an elevated temperature to 20 at least partially dehydrate the chromic sulphate and bind the fibers together in a coherent mass.

Heretofore, it has been the practice to employ 25 organic binding agents, such as starch, nitro-cellulose, oils, pitch and varnishes, as a binding agent for asbestos fibers, which agent also serves to cement the insulation to electric wires and cables. At high temperatures, these binding agents are not entirely 30 satisfactory because the organic material either decomposes or volatilizes and leaves the asbestos in a loose condition. In insulating material employed in such apparatus as electrical stoves, where high temperature is 35 encountered, this undesirable property of the organic binding agents is especially noticeable. The organic material is also inflammable and this factor increases the fire hazard when it is employed in connection with 40 inflammable material.

During my researches on this subject, I have discovered a suitable inorganic binding agent that is stable at elevated temperatures. I have found that, when chromic 45 sulphate is employed as a binding agent, the asbestos fibers will be bonded together permanently, even though the material is exposed to a high temperature, and this will be true even though some organic material 50 is present.

My invention is especially suitable for providing a flame-proof insulation for conductors because it avoids the necessity of utilizing an excessive amount of organic matter.

In practicing my invention, I employ 55 commercial chromic sulphate which is dissolved in water, preferably with the aid of heat, to obtain a solution containing a substantial amount of chromic sulphate, which is then allowed to cool. The asbestos is then immersed in, or drawn slowly through, the chromic-sulphate solution, drained and dried in an oven at a temperature of 150° C. to 60 300° C. for a sufficient length of time to at least partially dehydrate the sulphate. If 65 desired, the asbestos fibers may be bonded together by a small amount of an organic material and drawn through, or immersed in, the solution, or the asbestos may first be applied to electrical conductors and the coated conductors may then be drawn through, or immersed in, the solution.

As a result of the baking operation, the 70 commercial chromic sulphate, which, in its hydrated form, is soluble in water, becomes 75 practically insoluble, after being partially or completely dehydrated by baking.

The following specific example will serve 80 to explain and illustrate my invention. A Monel-metal stranded cable, having one 85 felted coat and one braided coat of asbestos was immersed in an aqueous solution containing 27.5% of chromic sulphate, by weight, for a period of two minutes. The cable was then removed and the surplus 90 chromic sulphate was allowed to drain off for three minutes. The cable was then baked in an oven for a period of one hour at a temperature of 150° C. In testing the insulation, it was found that it was capable of resisting 800 volts.

Since the amount of chromic sulphate in the solution may be varied widely, I do not desire to limit myself to any particular proportions. I have found that a solution 95 containing from 10% to 50%, by weight, of chromic sulphate is preferable. Furthermore, it is not necessary to employ water as the solvent, as other solvents may be 100 employed, such as alcohol or a mixture of

water and alcohol. However, for economical reasons, I prefer to utilize an aqueous solution of chromic sulphate as the impregnating medium.

5 The baking period may also be varied considerably and will be dependent upon the thickness of the impregnated material and the temperature. The time and temperature should be sufficient to, at least partially, dehydrate the chromic sulphate and to render it insoluble. At temperatures below 150° C., the chromic sulphate will not be dehydrated, while, if the temperature is raised above 300° C., the asbestos begins to disintegrate, and the chromic sulphate undergoes partial decomposition.

10 In some cases, the asbestos fibers may be held together by a small amount of a suitable binding agent, such as nitrocellulose, starch or dextrin. The material is then impregnated with chromic sulphate and baked at a sufficient temperature and for a sufficient length of time to eliminate the solvent, and, at least a portion of, the water of hydration. When it is desired to produce asbestos cemented together partially by an organic binder and partially by chromic sulphate, the baking 15 temperature must be maintained below the point of decomposition of the organic binder, which temperature, however, must be above the dehydration temperature of the chromic sulphate.

20 In preparing a material containing an organic material and chromic sulphate, the asbestos may be drawn through a solution containing chromic sulphate and starch or dextrin or both of such materials, and the impregnated material is baked at a temperature 25 above the dehydration temperature of the chromic sulphate but below the temperature of decomposition of the starch or dextrin, or, if desired, the fibers may be bound together by nitrocellulose and the 30 material passed through, or immersed in, a solution containing chromic sulphate and an organic material, such as starch or dextrin, or both of them, and the material allowed to drain. The impregnated asbestos is then 35 baked at a sufficient temperature and for a sufficient length of time to dehydrate the chromic sulphate and decompose the nitrocellulose without decomposing the starch or dextrin.

40 45 50 55 60 65 Dehydrated chromic sulphate is superior to sodium silicate as a binding agent, because it is a better insulator and is comparatively non-hygroscopic. In view of its amorphous characteristics, it is superior to a crystalline binding agent, because it forms a glass-like film that covers, and adheres to, the fabric. It adheres extremely well to the meshes of a fabric and is stable at temperatures at which organic binding agents 70 volatilize or decompose.

While I have described chromic sulphate as being especially suitable as a binding agent for asbestos when utilized as an insulation for electrical wires and cables, I do not desire to limit my invention in this respect, as the material may obviously be employed for various other purposes, such as for the brake bands of automobiles, for friction purposes, heating pads, or, in general, wherever asbestos is employed at the present time.

70 75 80 85 90 95 The term "asbestos", as employed in the specification and claims, refers to commercial asbestos which comprises asbestos fibers loosely held together by suitable means, such as cotton threads.

While I have described my invention in considerable detail and have given specific examples, it will be understood that the examples should be construed as illustrative and not by way of limitation, and, in view of the numerous modifications which may be effected therein, without departing from the spirit and scope of my invention, it is desired that only such limitations shall be imposed as are indicated in the appended claims.

I claim as my invention:

1. A composition of matter comprising asbestos fibers cemented together by a binding agent comprising chromic sulphate that is, at least partially, dehydrated.

2. A composition of matter comprising asbestos, an organic binding agent, and a chromic sulphate that is, at least partially, dehydrated.

3. An insulating material comprising asbestos fibers cemented together by a binding agent including chromic sulphate that is, at least partially, dehydrated.

4. An insulating material comprising asbestos fibers cemented together by a binding agent comprising an organic material and chromic sulphate that is, at least partially, dehydrated.

5. An article of manufacture consisting of a conductor coated with an insulating material comprising asbestos fibers cemented together by a binding agent including chromic sulphate that is, at least partially, dehydrated.

6. The method of binding asbestos fibers together which comprises immersing them in a solution containing chromic sulphate, withdrawing the material and then baking at a sufficient temperature to partially dehydrate the chromic sulphate.

7. The method of binding asbestos fibers together which comprises immersing them in a solution containing 10% to 50% chromic sulphate, by weight, withdrawing said material and then baking it at a temperature of from 150° C. to 300° C. for a sufficient length of time to, at least partially, dehydrate the sulphate.

8. The method of binding asbestos fibers together which comprises immersing them in an aqueous solution of chromic sulphate containing from 10% to 50%, by weight, of chromic sulphate, withdrawing the impregnated fibers and then baking at 150° C. to 300° C. for a sufficient length of time to, at least partially, dehydrate the chromic sulphate and bind the fibers together.

10 9. The method of binding asbestos fibers together which comprises impregnating them with an aqueous solution containing an organic binding agent and chromic sulphate, withdrawing the impregnated material, and 15 then baking at a temperature sufficient to, at least partially, dehydrate the sulphate.

10 10. In the method of binding asbestos fibers together, the step which comprises impregnating the fibers with a solution of chromic sulphate that is, at least partially, 20 dehydrated.

11. In the method of binding asbestos fibers together, the steps which comprise impregnating the fibers with chromic sulphate 25 and then heating to, at least partially, dehydrate the chromic sulphate.

12. The method of forming an insulated conductor which comprises felting or braiding asbestos around the conductor, impregnating the felted or braided material with a solution containing chromic sulphate, and then heating at a sufficient temperature to, 30 at least partially, dehydrate the chromic sulphate.

35 13. The method of forming an insulating material which comprises cementing asbestos fibers together by a binder that will be decomposed at a comparatively low temperature, impregnating the same with a solution containing chromic sulphate, and then heating at a sufficient temperature to decompose the organic binder and to, at least partially, 40 dehydrate the chromic sulphate.

In testimony whereof, I have hereunto 45 subscribed my name this 29th day of May, 1930.

LEON McCULLOCH.